

Aug. 14, 1945.

R. W. CAIRNS ET AL

2,382,130

TREATMENT OF NITROCELLULOSE

Filed May 19, 1943



FIG. 1



FIG. 3



FIG. 2



INVENTORS  
ROBERT W. CAIRNS  
RAPHAEL L. STERN

BY

*Cleveland B. Hollingshead*  
ATTORNEY

## UNITED STATES PATENT OFFICE

2,382,130

## TREATMENT OF NITROCELLULOSE

Robert W. Cairns, Wilmington, Del., and Raphael L. Stern, South River, N. J., assignors to Hercules Powder Company, Wilmington, Del., a corporation of Delaware

Application May 19, 1943, Serial No. 487,662

13 Claims. (Cl. 260—223)

This invention relates to a method for conditioning fibrous nitrated cellulose so that it may be stored safely without deterioration. It also relates to the product obtained by application of the method and to apparatus for carrying out the method.

Fibrous nitrated cellulose, especially the highly nitrated cellulose used for the preparation of smokeless powder, is maintained wet with water for safe storage before use and in transit. However, the nitrogen content of the wet nitrocellulose provides a condition which is conducive to growth of molds in the mass. Mold growths frequently spread in a short time through stored masses of nitrocellulose with consequent deterioration of the material.

In accordance with this invention, growth of molds in wet nitrated cellulose is prevented by distributing a lower aliphatic alcohol in the wet fibrous nitrated cellulose in a quantity to provide a solution of aqueous alcohol wetting the fibers, the solution having an average alcohol concentration between about 7% and about 45% by weight of the solution. The resulting product, i. e., fibrous nitrated cellulose wet with an aqueous alcohol solution in the range of concentration mentioned, may be stored with the same safety as nitrated cellulose wet only with water and, at the same time, it cannot deteriorate due to mold growth. The treated fibrous mass has the further advantage of being non-freezing or resistant to freezing, obviating thawing operations.

The method in accordance with this invention is carried out on stabilized fibrous nitrocellulose, wet with water, but usually freed of excess water such as by pressing or centrifuging. This material is placed in a container and treated to distribute an alcohol therein, most conveniently with the aid of apparatus which is a part of the present invention.

This apparatus is most readily described with reference to the drawing in which:

Figure 1 is a frontal view partly in section of the apparatus which includes a head and lance assembly for inserting the alcohol and means for operatively moving the assembly;

Figure 2 is a perspective view of the head and lance assembly; and

Figure 3 is a detailed view of a lance, partly in section.

Referring to Figure 1, which illustrates an apparatus in accordance with this invention in a position of use, it will be seen that the apparatus comprises a head 1 in which are mounted a plurality of lances 2. The lances are hollow contain-

ing a longitudinal passage 4 in each lance. The head is provided with an interior passage or passage system 5 which connects with the longitudinal passage of each of the lances. The head is also provided with an inlet fitting 6 leading to the passage system of the head and connected by a flexible conduit 7 to a pump or other source capable of providing a flow of the liquid to be distributed in the fibrous mass to the head passages. Figure 1 shows the lances in position extending into a barrel 8 which in normal operation is packed with the fibrous mass. The apparatus further comprises means for forcing the lances into the fibrous mass and then upon completion of the operation of distributing liquid in the mass, removing the lances. In the apparatus of Figure 1, this comprises a connecting rod 9 connecting the head to a piston 10 in a cylinder 11. The cylinder is provided with heads 12 provided with inlet and outlet fittings 13 connected to a suitable system for providing a fluid under pressure, and for arranging for release of the fluid as required to operate the piston, and thereby to lower and raise the head in which the lances are mounted with the force required for operation.

An arrangement of the plurality of lances is shown in Figure 2 which provides a bottom view in perspective of the head and lance assembly.

The particular assembly shown in Figure 2 comprises six lances in symmetrical arrangement supported by a circular head. Each lance is provided with a plurality of apertures 14 leading from the outer surface to the hollow passage of the lance.

The detailed construction of a suitable lance is shown in Figure 3. The lance consists of a rigid hollow tube provided with a sharp point and means for mounting the other end in the head. A plurality of holes 14 leading to the hollow passage permits escape of fluid forced into the hollow passage. The holes are spaced longitudinally along the lance and are placed on all sides of the lance. Preferably, the holes are spaced regularly and are at a distance, such as 3-6 inches from each other, to provide adequate distribution of liquid throughout the length of the lances. Preferably, the holes are countersunk using a relatively shallow wide cut around each hole. Countersinking is valuable in the prevention of clogging of the holes when operating with the fibrous nitrated cellulose since the nitrocellulose fibers readily cause plugging of ordinary drilled holes, due to their friable nature.

In operation, stabilized, washed, nitrated cellulose is placed in the water wet condition in a

container, such as a shipping barrel, and is packed therein in the usual manner. Preferably, the material is freed of excess water, for example by pressing or centrifuging. It is desirable to press or centrifuge the wet nitrocellulose to a known water content. The plurality of lances is then forced into the mass of fibrous nitrated cellulose and a known quantity of the alcohol is forced by pressure into the mass. The pressure utilized will be sufficient to force the alcohol into the lances and thence into the mass. It will usually be between about 25 pounds and about 200 pounds per square inch. At such a pressure, the desired quantity of the alcohol is distributed into the mass in a few seconds. The alcohol may be in pure form or in solution in water. The quantity of alcohol utilized is such that upon dilution by the water in the still wet mass, the solution resulting will have an average concentration between about 7% and about 45% by weight of alcohol of the solution.

Desirably, the water wet fibrous nitrated cellulose has a water content between about 15% and about 40% by weight prior to insertion of the alcohol. Sufficient alcohol or alcohol solution is then distributed in the mass to bring the concentration of the aqueous alcohol to 7-45% and to bring the total volatile content of the fibrous mass to between about 20% and about 45%, preferably between about 30% and about 40%.

The fibrous mass may contain more water than that mentioned at the beginning of the operation, if desired, and following the distribution therein of the amount of the alcohol required to obtain the desired concentration, excess solution may be removed, as by pressing or centrifuging, from the treated mass. However, this method is somewhat less convenient in view of the added operation involved.

The alcohol distributed in the mass shortly diffuses to form a solution with the water therein. The solution is substantially uniform in concentration. The concentration of the alcohol in the aqueous solution must be at least about 7% to prevent mold growth. The concentration should be no more than about 45% since at above this concentration, the safety in storage of water wet nitrocellulose decreases. Preferably, the concentration of the alcohol in the solution wetting the fibers is between about 20% and about 45% since this concentration is well removed from the border line of possible mold growth and since such concentration, in addition, gives the further advantage of lowering the freezing point of the mass to the range between about 13° F. and -27° F.

Ethyl alcohol is greatly preferred as the alcohol utilized for prevention of mold growth, since it is cheap and is usually utilized in later processing of the nitrated cellulose in the preparation of smokeless powder. However, other lower aliphatic water-soluble alcohols such as methyl alcohol, propyl alcohol, isopropyl alcohol, nitroethanol, and the like, may be used.

The method in accordance with this invention is particularly useful for conditioning fibrous nitrated cellulose having a nitrogen content between about 12.4 and 14.1%, this being the type used in smokeless powder manufacture, as such nitrated cellulose must be stored for safety wet with water. However, the method may also be applied to soluble fibrous nitrated cellulose types having a nitrogen content between about 10.5% and 12.4%.

What we claim and desire to protect by Letters Patent is:

1. The method of conditioning and preserving fibrous nitrated cellulose safely without substantial deterioration which comprises wetting the fibrous material with water containing in solution between about 7% and about 45% by weight of the solution of a lower aliphatic alcohol and storing the material wet with the said solution.
- 10 2. The method of conditioning and preserving fibrous nitrated cellulose safely without substantial deterioration which comprises wetting the fibrous material with water containing in solution between about 7% and about 45% by weight of the solution of ethyl alcohol, the water solution being in quantity between about 20% and about 45% by weight of the entire mass.
- 15 3. The method of preserving fibrous nitrated cellulose safely without substantial deterioration which comprises storing the fibrous nitrated cellulose wet with water containing in solution between about 7% and about 45% by weight of the solution of a lower aliphatic alcohol.
- 20 4. The method of preserving fibrous nitrated cellulose safely without substantial deterioration which comprises storing the fibrous nitrated cellulose wet with water containing in solution between about 7% and about 45% by weight of the solution of ethyl alcohol, the water solution being in a quantity between about 20% and about 45% by weight of the entire mass.
- 25 5. The method of conditioning and preserving fibrous nitrated cellulose safely without substantial deterioration which comprises forming a mass of the fibrous nitrated cellulose wet with essentially water, introducing a lower aliphatic water-soluble alcohol into the wet mass at a plurality of points in the mass in a quantity sufficient to form a solution containing between about 7% and about 45% of the alcohol upon dilution by the water, permitting the alcohol to diffuse in the mass and mix with the water therein to form a solution wetting the fibers having an average concentration between about 7% and about 45%, and storing the resulting fibrous nitrated cellulose.
- 30 6. The method of conditioning and preserving fibrous nitrated cellulose safely without substantial deterioration which comprises forming a mass of the fibrous nitrated cellulose wet with water in a quantity between about 15 and about 40% of the wet mass, introducing a lower aliphatic alcohol into the wet mass at a plurality of points in the mass in a quantity sufficient to increase the liquid content of the mass to between about 20% and about 45% of the resulting wet mass and to form a water solution in the mass having an average concentration of the alcohol by weight between about 7% and about 45% of the solution, permitting the alcohol to diffuse in the mass and to mix with the water therein, and storing the resulting fibrous nitrated cellulose.
- 35 7. The method of conditioning and preserving fibrous nitrated cellulose safely without substantial deterioration which comprises forming a mass of the fibrous nitrated cellulose wet with essentially water, introducing ethyl alcohol into the wet mass at a plurality of points in the mass in a quantity sufficient to form a solution containing between about 7% and about 45% of the alcohol upon dilution by the water, permitting the alcohol to diffuse in the mass and mix with the water therein to form a solution wetting the fibers having an average concentration
- 40
- 45
- 50
- 55
- 60
- 65
- 70
- 75

between about 7% and about 45%, and storing the resulting fibrous nitrated cellulose.

8. The method of conditioning and preserving fibrous nitrated cellulose safely without substantial deterioration which comprises forming a mass of the fibrous nitrated cellulose wet with water in a quantity between about 15 and about 40% of the wet mass, introducing ethyl alcohol into the wet mass at a plurality of points in the mass in a quantity sufficient to increase the liquid content of the mass to between about 20% and about 45% on the resulting wet mass and to form a water solution in the mass having an average concentration of the alcohol by weight between about 7% and about 45% of the solution, permitting the alcohol to diffuse in the mass and to mix with the water therein, and storing the resulting fibrous nitrated cellulose.

9. A mass of fibrous nitrated cellulose suitable for safe prolonged storage consisting essentially of nitrated cellulose fibers wet with water containing in solution between about 7% and about 45% by weight of the solution of a lower aliphatic alcohol.

10. A mass of fibrous nitrated cellulose suitable for safe prolonged storage consisting essentially of nitrated cellulose fibers wet with water containing in solution between about 7% and about 45% by weight of the solution of ethyl alcohol.

11. A mass of fibrous nitrated cellulose suitable for safe prolonged storage consisting essentially of nitrated cellulose fibers wet with water containing in solution between about 7% and about 45% by weight of the solution of a lower aliphatic alcohol, the said mass containing between about 20% and about 45% by weight of the water solution.

12. A mass of fibrous nitrated cellulose suitable for safe prolonged storage consisting essentially of nitrated cellulose fibers wet with water containing in solution between about 7% and about 45% by weight of the solution of ethyl alcohol, the said mass containing between about 20% and about 45% by weight of the water solution.

13. The method of conditioning and preserving fibrous nitrated cellulose safely without substantial deterioration which comprises wetting the fibrous material with water containing in solution between about 7% and about 45% by weight of the solution of a lower aliphatic alcohol, the water solution being of substantially uniform concentration throughout the fibrous material, and storing the material wet with the said solution.

ROBERT W. CAIRNS.  
RAPHAEL L. STERN.